

## UNITED STATES PATENT OFFICE

2,111,823

## PROCESS OF TREATING HIDES AND SKINS

Christoph Thomsen, Alfred Eckelmann, and  
Ernst Koch, Frankfort-on-the-Main, Ger-  
many, assignors to I. G. Farbenindustrie Ak-  
tengesellschaft, Frankfort-on-the-Main, Ger-  
many

No Drawing. Application December 17, 1935,  
Serial No. 54,944. In Germany December 22,  
1934

4 Claims. (Cl. 149—1)

The present invention relates to a process of  
treating hides and skins.

We have found that hides and skins are im-  
proved by a treatment with basic compounds,  
5 containing nitrogen and having a straight or  
branched, saturated or unsaturated carbon  
chain of at least 5 carbon atoms, or a hydro-  
aromatic ring containing at least 5 members, in  
10 the form of their addition salts. The carbon  
chain may be interrupted by other atoms or atom  
groups such as, for instance, by O, S, N, CO,  
CONH, but at least 5 carbon atoms must directly  
be connected with each other. The substitution  
products and derivatives of these bodies may  
15 also be used.

As such compounds there may, for instance,  
be named: primary, secondary and tertiary  
amines, aminoxydes, imidazoles, imidazolines,  
pyrimidines; furthermore imidoethers, imidothio-  
ethers and amidines, the last three obtainable,  
20 for instance, according to the co-pending U. S.  
application Serial No. 751,252 and 751,253, filed  
November 2, 1934, in the name of Alfred Eckel-  
mann and Ernst Koch, furthermore substituted  
ureas, thioureas, guanidines and carbaminic acid  
25 esters.

There may be used, for instance, the addition  
salts of the following bodies: octylamine, do-  
decylamine, stearylamine, the technical fatty  
30 amines such as, for instance, mixtures of amines  
prepared from coco-nut oil fatty acid, palm nut  
oil fatty acid or from technical stearic acid, the  
amines made from technical montanic acid or  
naphthenic acid, abietylamine, paraoctylaniline,  
35 monomethylstearylamine, octylglucamine, mono-  
oleylhydroxy-propylenediamine, stearoyldiethyl-  
enediamine, decylhexahydrophenylamine, N-  
octylaniline, N-stearyl-para-phenylenediamine,  
N-dodecylaphthylamine, dodecylfurfurylamine,  
40 dimethyldodecylamine, dodecylmethylglucamine,  
asymmetric ethyloctylethylenediamine, N-di-  
octylaniline, dimethyldodecylamineoxide; fur-  
thermore N-methylstearbenzimidazole, N-do-  
decylacetbenzimidazole, N-stearoylhydroxyethyl-  
45 acetbenzimidazole, laurimidazoline, N-dodecyl-  
pyrimidine, stearimidomethylether, laurimido-  
butylether, the imidoisobutylether of coco-nut  
oil fatty acid, benzimidodecylether, acetimidido-  
stearyl ether, stearimidomethylthioether, stear-  
50 amide, the amide of palm nut oil fatty acid,  
symmetrical and asymmetrical steardiethyl-  
amide, steardietethylamino-ethylamide, stear-  
oxethylamide, mono-stearylurea, asymmetrical  
dodecylaminoethylurea, asymmetrical decyl-  
55 methylolurea, N-stearyl-N'-diethylaminoethyl-

urea, dodecylthiourea, symmetrical dioctyl-  
guanidine, diethylaminoethylcarbaminic acid  
stearyl ester, N-dodecylpiperidine, beta-stearyl-  
aminopyridine. As salts there may be used, for  
instance, the chlorides, sulfates, formates or ace-  
tates of these bodies.

There may also be used the mixtures of these  
products with each other or with other products,  
for instance: mixtures of stearimidomethyl ether  
hydrochloride and stearamidine hydrochloride or  
10 stearimidazoline hydrochloride, or mixtures of  
dodecylurea with steardiethylamide hydro-  
chloride, of stearic acid diethylamide with stear-  
amidine hydrochloride.

Insofar as these bodies are liquid, they may  
be used without application of solvents, other-  
wise they may suitably be used in the form of  
an aqueous solution, or in case they are not  
sufficiently soluble in water in the form of an  
15 emulsion. If necessary, they may be applied in  
conjunction with organic solvents, oils and the  
like or with dispersing agents.

The said products are well absorbed by hide  
and skin. They may be applied before or dur-  
ing the tanning process. The leathers and furs  
20 which have been prepared from hides and skins  
either pre-treated with the said products or in  
the presence of the said products, show an  
agreeable soft feel. The tanning process takes  
place more uniformly and more rapidly. The  
25 products, furthermore, prevent in many cases  
deleterious influences on the fiber, and, with the  
aid of these products there may be obtained  
leathers of very good resistance to tearing. Since  
many of these products are fast to light, they  
30 may be used with great advantage for the manu-  
facture of leathers fast to light, especially white  
leathers. The products may also be used for  
treating such hides and skins which are not in-  
tended to be worked up immediately, for in-  
35 stance, by tanning. The products have a pre-  
serving action and prevent the fiber from being  
detrimentally affected; furthermore it has  
proved in many cases that the skins or hides thus  
40 treated may again very easily be soaked, if  
necessary with addition of other soaking agents.

The following examples serve to illustrate the  
invention, but they are not intended to limit it  
thereto; the parts are by weight:

(1) 50 parts of calf skin are drummed in an  
aqueous solution of 125 parts of water and 10  
parts of the diethylamidine hydrochloride, pre-  
pared from commercial stearic acid until the  
skin has absorbed a sufficient quantity of the  
50 product. 3 parts of a formaldehyde solution of  
55

30 per cent. strength are now added to the solution and the skin is subsequently drummed for 5 hours. The leather is then washed and dried in the usual manner. The leather thus obtained is 5 white and fast to light and possesses a high resistance to tearing.

(2) 100 parts of sheep skin are drummed for 10 hours in a solution which contains per liter of liquor 100 parts of amidine hydrochloride, prepared from the nitrile of coco-nut oil fatty acid, and 25 parts of formaldehyde solution of 30 per cent. strength. The skin is well washed and dried in the usual manner. The leather obtained has the properties of that described in 15 Example 1.

(3) 100 parts of pickled goat skin are well drummed for 5 hours in an aqueous solution of 150 parts of water and 3 parts of benzoquinone and treated in a fresh liquor containing the imidazoline hydrochloride prepared from commercial stearic acid. The leather may advantageously be 20 after-treated in the usual manner.

(4) 80 parts of well de-limed sheep skin are treated in a solution which contains per liter of liquor 70 parts of imidomethyl-ether hydrochloride prepared from technical stearic acid, 50 parts of the product of the reaction of oleic acid chloride on methyl-taurine and 15 parts of a formaldehyde solution of 30 per cent. strength.

(5) 100 parts of calf skin are drummed for 20 hours in an aqueous solution of 250 parts of water, 5 parts of lauramidine hydrochloride and 5 parts of benzoquinone. A brown soft leather is obtained which resists tearing.

(6) 80 parts of calf skin are first pre-treated with a solution of 8.5 parts of the diethylamidine hydrochloride prepared from commercial stearic acid and 3.5 parts of dodecylurea in 250 parts of water. Later on, 3 parts of acetaldehyde are 40 added to this liquor and the skin is then after-drummed for a short time. A soft, feebly yellow leather of very good resistance to tearing is obtained.

(7) 50 parts of prepared rabbit skin are treated 45 with an aqueous solution consisting of 100 parts of water and 10 parts of unsymmetrical diethylamidine hydrochloride prepared from technical stearic acid, until the skin has absorbed enough of the product. The skin is then after-treated 50 with a formaldehyde solution of 3 per cent. strength. A soft fur is obtained which has a very good resistance to tearing.

(8) 100 parts of cow hide are shaken for 3 days with 300 parts of water, containing 10 parts 55 of the diethylaminoethylamidine hydrochloride prepared from commercial stearic acid; thereupon the hide is rinsed for a short time and tanned with a tanning agent prepared according to German Patent No. 436,446 from colophonium-cresol. The pre-treatment essentially enhances the fastness to tearing of the leather.

(9) 75 parts of calf skin are shaken for 3 days with a solution of 7.5 parts of stearoyldiethyl-60 ylenediamine hydrochloride in 200 parts of water. The leather is then rinsed and shaken with 300 parts of a solution which contains 15 parts of ammoniacal iron alum. To this tanning solution there are added in three equal portions and 65 in intervals of 3 hours 75 parts of a sodium acetate solution of 10 per cent. strength. The leather is then shaken for a further 2 days, thereupon rinsed and dried. The leather is very well and uniformly tanned, is not streaky in the 70 cut, has a full and soft feel, a good resistance 75

to tearing and shows only a feeble tendency to grain-cracking.

We claim:

1. The process which comprises treating untanned hides and skins with the salts of basic compounds selected from the group consisting of compounds of the general formula:



and of the general formula:



and of the general formula:



wherein X stands for  $\text{OR}_1$  or  $\text{SR}_1$ ; R,  $\text{R}_1$ ,  $\text{R}_2$  and  $\text{R}_3$  being members of the group consisting of hydrogen, aliphatic radicals with a straight chain, aliphatic radicals with a branched chain and radicals having a cyclo-aliphatic ring, at least one of the substituent radicals in said basic compound containing at least 5 carbon atoms.

2. The process which comprises treating untanned hides and skins with the salts of amidines of the general formula:



R,  $\text{R}_1$ ,  $\text{R}_2$  and  $\text{R}_3$  being members of the group consisting of hydrogen, aliphatic radicals with a straight chain, aliphatic radicals with a branched chain and radicals having a cyclo-aliphatic ring, at least one of them having at least 5 carbon atoms.

3. The process which comprises treating untanned hides and skins with asymmetric diethylamidine-hydrochloride, derived from commercial stearic acid.

4. Hides and skins, which have been improved by treating the untanned materials with the salts of basic compounds selected from the group consisting of compounds of the general formula:



and of the general formula:



and of the general formula:



wherein X stands for  $\text{OR}_1$  or  $\text{SR}_1$ ; R,  $\text{R}_1$ ,  $\text{R}_2$  and  $\text{R}_3$  being members of the group consisting of hydrogen, aliphatic radicals with a straight chain, aliphatic radicals with a branched chain and radicals having a cyclo-aliphatic ring, at least one of the substituent radicals in said basic compound containing at least 5 carbon atoms.

CHRISTOPH THOMSEN.  
ALFRED ECKELMANN.  
ERNST KOCH.